

## UNITED STATES PATENT OFFICE.

MARCEL MELLIAND, OF MANNHEIM, GERMANY, ASSIGNOR TO MELIANA CORPORATION OF AMERICA, A CORPORATION OF NEW YORK.

## PROCESS OF TREATING VEGETABLE FIBERS AND FABRICS.

No Drawing. Application filed July 25, 1927, Serial No. 208,404, and in Germany June 25, 1926.

This invention relates to the improvement of material comprising vegetable fiber, and in particular to such improvement effected by means of a treatment with strong hot 5 solutions of caustic alkalies either alone or in conjunction with one or more mercerizing treatments, and to the improved materials thereby produced.

The improvement of fabrics composed of 10 vegetable fiber, such as cotton, by treatment with strong caustic alkalies, consists in a more or less extensive structural alteration of the material, which is in general combined with a morphological, chemical or physio- 15 chemical change in its composition. All the processes in which a treatment with cold caustic alkalies is used for this purpose are today designated as "mercerization", without any particular reference to the use of a 20 certain tension or of pre- or post-treatment, in case only the structural changes of increased lustre and solidity, or the chemical change of the formation of hydrocelluloses, and thereby a better and more economical 25 absorption of dyestuffs, are produced.

An extension of this operation to the products obtained by treatments with strong acids (amylization) is occasionally technically useful, but is not scientifically justifiable, unless it is expressly intended to work 30 with a material already containing hydrocelluloses or the amylied material is to be submitted to a subsequent mercerization. It is well known that mercerization can be 35 carried out repeatedly and with variations of the working conditions. Thus durable, bicolored crepes can be produced advantageously by printing caustic alkali upon mercerized goods. The so-called "acid mer- 40 cerization" should be designated as a combination process. It is not yet clear what products are formed by these treatments, which Thies calls "progressive mercerization". They all, however, give the fiber and 45 the fabric a characteristic stiffness, with a decrease in elasticity and an increase in the tendency to wrinkle. Thies (Newzeitliche Waschprozesse, Ed. 2, page 11) also found that because of the formation of degrada- 50 tion products the fibers show no increased resistance in washing in spite of the apparently increased solidity.

I have now found that by treating material comprising vegetable fiber, such for 55 instance as cotton fabrics, with strong, hot

to boiling, caustic alkalies, e. g., NaOH solution of about 50° Bé., without tension, that hitherto unknown effects are produced, the strength and elasticity of the fibers being raised and their curliness being increased. 60 The time of treatment is adapted to the materials treated and to the desired character of the product, and the treatment is stopped immediately after the intended changes, structural and otherwise, have occurred. 65 These conditions are further described below.

The above described process will be briefly designated as melianization. The materials treated by this process completely retain 70 their character and their valuable properties in the wash. In particular they undergo no further shrinkage as do the above-mentioned hitherto known products, as well as most textile materials. A strikingly small ten- 75 dency toward wrinkling is also characteristic of all "melianized" products.

In the present state of the art, every technician, when once apprised thereof, will soon discover in the suitable application of 80 the principles given by me, that, analogous to the course of events in mercerization, in melianization the alterations, structural and otherwise, take place very quickly, that is, in fractions of minutes or at most in a few 85 minutes. If the reaction is not stopped at this point, not only is the desired result partly or wholly nullified, but the cellulose is also harmed by the rapid attack of the 90 treating liquor on the inner substance of the fiber. The necessity for an immediate stopping of the reaction has not been recognized heretofore, although the manner in which this process should be carried out in various 95 cases is governed by the general rules relating to the breaking off of reactions in which the critical point is dependent on both temperature and concentration.

If a loosely woven fabric is melianized by treatment with strong caustic alkalies at tem- 100 peratures from 60° to 100° C., or even higher, a great swelling of the fibers takes place together with a characteristic curling of the fibers, and the result is an extremely soft material similar to wool. The reaction 105 should be stopped when the curling effect is large compared with the change in count of the yarn and when the threads or the fabric take on a smoothness without a noteworthy increase in the luster. In agreement with 110

this appearance chemical investigation shows no hydrocelluloses, or at most a very small amount, and never shows the presence of any oxycelluloses. On the other hand, if 5 a closely woven fabric is melianized the curling effect is somewhat less compared with the change in count. The fabric shows an increased flexibility and pliancy but no noteworthy wool characteristics.

10 I have further found that, starting, for instance, with various cotton fabrics, I can obtain, according to the conditions used, varied but highly valuable materials, which often possess a striking linen or silk character, 15 by combining with the above-described "melianizing" treatment, one or more additional treatments resembling the well-known mercerization process. These materials likewise have the desirable properties of retaining their characteristics in the wash, undergoing no further shrinkage and having a very slight tendency to wrinkle.

When I treat the above-mentioned raw materials in the cold with strong caustic 25 alkalies after a previous melianization I obtain, according to the raw material and its previous treatment, materials of striking beauty of the character of linen and silk. Similar products are obtained when normally mercerized materials are melianized. In general, however, it may be said that the treatment with cold alkali after the melianization is better in most cases. In this way the desired effects are obtained with most 30 goods without the application of any special tension. In the case of many materials a simple saturation with the cold alkali is sufficient.

40 *Examples.*

45 *Wash silk.*—An ordinary cotton muslin is prepared by mercerization in the usual way. Then the material is treated with 43% caustic soda at 92° C. for 3 minutes without tension, the caustic is immediately, after the structural change, driven out with boiling water, and, in case the result is not yet completely satisfactory, the material is impregnated with caustic soda solution for a short time and this is removed without tension. If stronger caustic solutions, e. g., of 50% NaOH, are used for the melianization the feel is somewhat fuller.

55 *Linen.*—Ordinary grey cotton goods is neither singed, desized, nor bleached, but treated with hot water, then treated for five minutes with 60% caustic soda solution at 88° C., without tension, thoroughly washed, given a short continuous chlor in the width, led through 23° Bé. caustic soda solution at 18° C. for a few minutes without tension, and washed out. A material is obtained of the typical character of a 3/4 white linen. An improvement in the feel may sometimes

be obtained by a treatment in a soaping bath 65 and souring with an organic acid.

In the application of the processes of this invention the melianizing operation can be carried out with strong caustic alkali solutions ranging from about 20° to about 70° 70 Bé., at temperatures of from about 60° C. to the boiling point of the solutions and the time of treatment will in general be from 1 to 5 minutes.

The term "cold caustic alkali solutions" 75 as used in the specification and claims is intended to denote such solutions at ordinary temperatures not lower than 0° C.

It will thus be evident that the present invention contemplates the treatment of materials comprising vegetable fibers by the above described melianizing operation alone or in combination with any of the known mercerizing operations.

The present application is a continuation- 85 in-part of my application Ser. No. 117,643, filed June 21, 1926.

I claim:

1. A process for treating cotton fabrics, which comprises subjecting said materials 90 to the action of strong hot solutions of caustic alkalies for a short time, without tension, in combination with at least one mercerizing treatment.

2. A process for treating cotton fabrics, 95 which comprises subjecting said materials to the action of strong hot solutions of caustic alkalies for a short time, without tension, in combination with at least one treatment with cold caustic alkali solution.

3. A process for treating cotton fabrics, which comprises subjecting said materials to the action of a solution of a caustic alkali of from 20° Bé. to 70° Bé. at from 60° C. to the boiling point of the solution for from 105 1 to 5 minutes without tension, in combination with at least one mercerizing treatment.

4. A process for treating cotton fabrics, which comprises subjecting said materials 110 to the action of a solution of caustic alkali of from 20° Bé. to 70° Bé. at from 60° C. to the boiling point of the solution for from 1 to 5 minutes without tension, and thereafter treating the materials with cold caustic alkali for a short time.

5. As a new produce, cotton fabric which is highly elastic and flexible, the fibers thereof being strongly curled, said characteristics being permanent, particularly to washing and boiling, which fabric is made by 120 treating a cotton fabric with a solution of a caustic alkali of from 20° Bé. to 70° Bé. at from 60° C. to 100° C. for from 1 to 5 minutes without tension, in combination with at least one treatment with cold caustic alkali 125 solution.

In testimony whereof, I affix my signature.  
MARCEL MELLAND,